



US006679956B2

(12) **United States Patent**  
**Bhargava**

(10) **Patent No.:** **US 6,679,956 B2**  
(b4) **Date of Patent:** **\*Jan. 20, 2004**

(54) **PROCESS FOR MAKING COPPER-TIN-ZINC ALLOYS**

(75) Inventor: **Ashok K. Bhargava**, Cheshire, CT (US)

(73) Assignee: **Waterbury Rolling Mills, Inc.**, Waterbury, CT (US)

(\*) Notice: Subject to any disclaimer, the term of this patent is extended or adjusted under 35 U.S.C. 154(b) by 14 days.

This patent is subject to a terminal disclaimer.

(21) Appl. No.: **09/808,337**

(22) Filed: **Mar. 14, 2001**

(65) **Prior Publication Data**

US 2001/0010243 A1 Aug. 2, 2001

**Related U.S. Application Data**

(60) Continuation-in-part of application No. 09/527,144, filed on Mar. 16, 2000, which is a continuation of application No. 09/103,866, filed on Jun. 24, 1998, now Pat. No. 6,099,663, which is a division of application No. 08/931,696, filed on Sep. 16, 1997, now Pat. No. 5,893,953.

(51) **Int. Cl.**<sup>7</sup> ..... **C22F 1/08**

(52) **U.S. Cl.** ..... **148/554; 148/680; 148/681; 148/682; 148/683; 148/684; 148/685**

(58) **Field of Search** ..... **148/554, 680, 148/681, 682, 684, 685**

(56) **References Cited**

**U.S. PATENT DOCUMENTS**

|             |         |                 |
|-------------|---------|-----------------|
| 3,923,558 A | 12/1975 | Shapiro et al.  |
| 4,586,967 A | 5/1986  | Shapiro et al.  |
| 4,605,532 A | 8/1986  | Knorr et al.    |
| 4,627,960 A | 12/1986 | Nakajima et al. |
| 4,666,667 A | 5/1987  | Kamio et al.    |

|             |           |                                |
|-------------|-----------|--------------------------------|
| 4,822,562 A | 4/1989    | Miyafuji et al.                |
| 4,935,076 A | 6/1990    | Yamaguchi et al.               |
| 4,971,758 A | 11/1990   | Suzuki et al.                  |
| 5,002,732 A | 3/1991    | Yamasaki et al.                |
| 5,024,814 A | 6/1991    | Futatasuka et al. .... 420/473 |
| 5,508,001 A | 4/1996    | Suzuki et al.                  |
| 5,624,506 A | 4/1997    | Tsuzaki et al. .... 148/433    |
| 5,853,505 A | * 12/1998 | Brauer et al. .... 148/433     |
| 5,893,953 A | * 4/1999  | Bhargava ..... 148/685         |
| 5,916,386 A | * 6/1999  | Bhargava ..... 148/554         |
| 6,099,663 A | 8/2000    | Bhargava                       |

**FOREIGN PATENT DOCUMENTS**

|    |           |          |
|----|-----------|----------|
| JP | 62-116745 | 5/1987   |
| JP | 03-294461 | 4/1990   |
| JP | 3-002341  | 1/1991   |
| JP | 03199357  | * 8/1991 |
| JP | 06-073474 | 8/1992   |
| JP | 06-220594 | 1/1993   |
| JP | 62-182240 | 9/1993   |
| JP | 63-161134 | 9/1993   |
| JP | 6-184679  | 7/1994   |
| JP | 6-184678  | 9/1994   |
| JP | 6-299275  | 10/1994  |
| JP | 6-220594  | 11/1994  |
| JP | 10-130755 | 11/1996  |

\* cited by examiner

*Primary Examiner—Sikyin Ip*

(74) *Attorney, Agent, or Firm—Wiggin & Dana LLP; William A. Simons; Michael K. Kinney*

(57) **ABSTRACT**

A process for making a copper base alloy comprises the steps of casting a copper base alloy containing tin, zinc, iron and phosphorous and forming phosphide particles uniformly distributed throughout the matrix. The forming step comprises homogenizing the alloy at least once for at least one hour at a temperature from 1000 to 1450° F., rolling to final gauge including at least one process anneal for at least one hour at 650 to 1200° F. followed by slow cooling, and stress relief annealing at final gauge for at least one hour at 300 to 600° F.

**15 Claims, No Drawings**

**PROCESS FOR MAKING COPPER-TIN-ZINC  
ALLOYS**

**CROSS-REFERENCE TO RELATED  
APPLICATION(S)**

This application is a continuation-in-part of U.S. Ser. No. 09/527,144, filed Mar. 16, 2000, entitled COPPER ALLOY AND PROCESS FOR OBTAINING SAME, which is a continuation of U.S. Ser. No. 09/103,866, filed Jun. 24, 1998, entitled COPPER ALLOY AND PROCESS FOR OBTAINING SAME, now U.S. Pat. No. 6,099,663, issued Aug. 8, 2000, which is a divisional of U.S. Ser. No. 08/931,696, filed Sep. 16, 1997, entitled COPPER ALLOY AND PROCESS FOR OBTAINING SAME, now U.S. Pat. No. 5,893,953, issued Apr. 13, 1999.

**BACKGROUND OF THE INVENTION**

The present invention relates to copper base alloys having utility in electrical applications and to a process for producing said copper base alloys.

There are a number of copper base alloys that are used in connector, lead frame and other electrical applications because their special properties are well suited for these applications. Despite the existence of these alloys, there remains a need for copper base alloys that can be used in applications that require high yield strength greater than 80 KSI, together with good forming properties that allow one to make 180° badway bends with a R/T ratio of 1 or less plus low relaxation of stress at elevated temperatures and freedom of stress corrosion cracking. Alloys presently available do not meet all of these requirements or have high costs that make them less economical in the marketplace or have other significant drawbacks. It remains highly desirable to develop a copper base alloy satisfying the foregoing goals.

Beryllium copper generally has very high strength and conductivity along with good stress relaxation characteristics; however, these materials are limited in their forming ability. One such limitation is the difficulty with 180° badway bends. In addition, they are very expensive and often require extra heat treatment after preparation of a desired part. Naturally, this adds even further to the cost.

Phosphor bronze materials are inexpensive alloys with good strength and excellent forming properties. They are widely used in the electronic and telecommunications industries. However, they tend to be undesirable where they are required to conduct very high current under very high temperature conditions, for example under conditions found in automotive applications for use under the hood. This combined with their high thermal stress relaxation rate makes these materials less suitable for many applications.

High copper, high conductivity alloys also have many desirable properties, but generally do not have mechanical strength desired for numerous applications. Typical ones of these alloys include, but are not limited to, copper alloys 110, 122, 192 and 194.

Representative prior art patents include U.S. Pat. Nos. 4,666,667, 4,627,960, 2,062,427, 4,605,532, 4,586,967, 4,822,562, and 4,935,076.

Accordingly, it is highly desirable to develop copper base alloys having a combination of desirable properties making them eminently suitable for many applications.

**SUMMARY OF THE INVENTION**

In accordance with the present invention, it has been found that the foregoing objective is readily obtained.

Copper base alloys in accordance with the present invention consist essentially of tin, phosphorous, iron, zinc, and the balance essentially copper. It is particularly advantageous to include nickel and/or cobalt in the alloy. Alloys in accordance with the present invention may also include aluminum, silver, boron, beryllium, calcium, chromium, indium, lithium, magnesium, manganese, lead, silicon, antimony, titanium, and zirconium. As used herein, the percentages are weight percentages.

It is desirable and advantageous in the alloys of the present invention to provide phosphide particles of iron and/or nickel and/or magnesium or a combination thereof, uniformly distributed throughout the matrix since these particles serve to increase strength, conductivity, and stress relaxation characteristics of the alloys. The phosphide particles may have a particle size of 50 Angstroms to about 0.5 microns and may include a finer component and a coarser component. The finer component may have a particle size ranging from about 50 to 250 Angstroms, preferably from about 50 to 200 Angstroms. The coarser component may have a particle size generally from 0.075 to 0.5 microns, preferably from 0.075 to 0.125 microns.

The alloys of the present invention enjoy a variety of excellent properties making them eminently suitable for use as connectors, lead frames, springs and other electrical applications. The alloys should have an excellent and unusual combination of mechanical strength, formability, thermal and electrical conductivities, and stress relaxation properties.

The process of the present invention comprises: casting a copper base alloy having a composition as aforesaid; homogenizing at least once for at least one hour at temperatures from about 1000 to 1450° F.; rolling to finish gauge including at least one process anneal for at least one hour at 650 to 1200° F.; and stress relief annealing for at least one hour at a temperature in the range of 300 to 600° F., thereby obtaining a copper alloy including phosphide particles uniformly distributed throughout the matrix. Nickel and/or cobalt may be included in the alloy as above.

**DETAILED DESCRIPTION OF THE  
PREFERRED EMBODIMENT(S)**

The alloys of the present invention are modified copper-tin-zinc alloys. They are characterized by higher strengths, better forming properties, higher conductivity, and stress relaxation properties that represent a significant improvement over the same properties of the unmodified alloys.

The alloys in accordance with the present invention include those copper base alloys consisting essentially of tin in an amount from about 0.1 to 4.0%, preferably in an amount from about 1.5% to 4.0% and most preferably from about 2.5 to 4.0%, phosphorous in an amount from about 0.01 to about 0.35%, preferably from about 0.01 to about 0.2%, iron in an amount from about 0.01 to about 0.8%, preferably from about 0.05 to about 0.8%, zinc in an amount from about 0.1 to about 15%, preferably from about 1.0 to 15%, and most preferably in an amount from about 1.0% to less than 9.0%, and the balance essentially copper. These alloys typically will have phosphide particles uniformly distributed throughout the matrix.

These alloys may also include nickel and/or cobalt in an amount up to about 0.5% each, preferably from about 0.001 to about 0.5% of one or combinations of both.

One may include one or more of the following elements in the alloy combination: aluminum, silver, boron, beryllium, calcium, chromium, indium, lithium, magnesium,

manganese, lead, silicon, antimony, titanium, and zirconium. These materials may be included in amounts less than 0.1%, each generally in excess of 0.001 each. The use of one or more of these materials improves the mechanical properties such as stress relaxation properties; however, larger amounts may affect conductivity and forming properties.

The aforesaid phosphorous addition allows the metal to stay deoxidized making it possible to cast sound metal within the limits set for phosphorous, and with thermal treatment of the alloys, phosphorous forms a phosphide with iron and/or iron and nickel and/or iron and magnesium and/or a combination of these elements, if present, which significantly reduces the loss in conductivity that would result if these materials were entirely in solid solution in the matrix. It is particularly desirable to provide iron phosphide particles uniformly distributed throughout the matrix as these help improve the stress relaxation properties by blocking dislocation movement.

Iron in the range of about 0.01 to about 0.8% and particularly about 0.05 to about 0.25% increases the strength of the alloys, promotes a fine grain structure by acting as a grain growth inhibitor and in combination with phosphorous in this range helps improve the stress relaxation properties without negative effect on electrical and thermal conductivities.

Nickel and/or cobalt in an amount from about 0.001 to 0.5% each and preferably 0.01 to 0.3% each, are desirable additives since they improve stress relaxation properties and strength by refining the grain and through distribution throughout the matrix, with a positive effect on the conductivity.

Zinc helps deoxidize the alloy, helping the castings to be sound without use of excessive phosphorous that can hurt conductivities. Zinc also helps in keeping the metal oxide free for good adhesion in plating.

The process of the present invention includes casting an alloy having a composition as aforesaid. Any suitable casting technique known in the art such as horizontal continuous casting may be used to form a strip having a thickness in the range of from about 0.500 to 0.750 inches. The processing includes at least one homogenization for at least one hour, and preferably for a time period in the range of from about 1 to about 24 hours, at temperatures in the range of from about 1000 to 1450° F. At least one homogenization step may be conducted after a rolling step. After homogenization, the strip may be milled once or twice to remove from about 0.020 to 0.100 inches of material from each face.

The material is then rolled to final gauge, including at least one process anneal at 650 to 1200° F. for at least one hour and preferably for about 1 to 24 hours, followed by slow cooling to ambient at 20 to 200° F. per hour.

The material is then stress relief annealed at final gauge at a temperature in the range of 300 to 600° F. for at least one hour and preferably for a time period in the range of about 1 to 20 hours. This advantageously improves formability and stress relaxation properties.

The thermal treatments advantageously and most desirably provide the alloys of the present invention with phosphide particles of iron and/or nickel and/or magnesium or a combination thereof uniformly distributed throughout the matrix. The phosphide particles increase the strength, conductivity, and stress relaxation characteristics of the alloys. The phosphide particles may have a particle size of about 50 Angstroms to about 0.5 microns and may include a finer component and a coarser component. The finer component may have a particle size of about 50 to 250

Angstroms, preferably from about 50 to 200 Angstroms. The coarser component may have a particle size generally from 0.075 to 0.5 microns, preferably from 0.075 to 0.125 microns.

Alloys formed in accordance with the process of the present invention and having the aforesaid compositions are capable of achieving a yield strength in the 80–100 ksi range with bending ability at a radius equal to its thickness, badway, on a width up to 10 times the thickness. Additionally, they are capable of achieving an electrical conductivity of the order of 35% IACS, or better. The foregoing coupled with the desired metallurgical structure should give the alloys a high stress retention ability, for example over 60% at 150° C., after 1000 hours with a stress equal to 75% of its yield strength on samples cut parallel to the direction of rolling, and makes these alloys very suitable for a wide variety of applications requiring high stress retention capabilities. Moreover, the present alloys do not require further treatment by stampers.

This invention may be embodied in other forms or carried out in other ways without departing from the spirit or essential characteristics thereof. The present embodiments are therefore to be considered as in all respects illustrative and not restrictive, the scope of the invention being indicated by the appended claims, and all changes which come within the meaning and range of equivalency are intended to be embraced therein.

What is claimed is:

1. A process for making a copper base alloy which comprises the steps of:

casting a copper base alloy containing tin, zinc, iron and phosphorous;

forming phosphide particles uniformly distributed throughout the matrix of said alloy;

said forming step comprising homogenizing said alloy at least once for at least one hour at a temperature from 1000 to 1450° F., rolling to final gauge including at least one process anneal for at least one hour at 650 to 1200° F. followed by slow cooling, and stress relief annealing at final gauge for at least one hour at 300 to 600° F.;

wherein said phosphide particle forming step comprises forming phosphide particles having a finer component having a particle size in the range of from about 50 to 250 Angstroms and a coarser component having a particle size from 0.075 microns to 0.5 microns.

2. Process according to claim 1, wherein said finer phosphide particles have a particle size in the range of from about 50 to 200 Angstroms and said coarser phosphide particles have a particle size in the range from 0.075 microns to 0.125 microns.

3. Process according to claim 1, wherein said iron and said phosphorous are present in said copper base alloy in an amount to form iron phosphide particles uniformly distributed through the matrix of the copper base alloy to block dislocation movement and thereby help improve stress relaxation properties of said alloy.

4. Process according to claim 3, wherein said iron is present in an amount from about 0.01 to 0.8% by weight and said phosphorous is present in an amount from 0.0 1% to 0.35% by weight.

5. Process according to claim 1, further comprising refining alloy grain by adding at least one of nickel and cobalt in an amount from about 0.001 to 0.5% each to said copper base alloy prior to said casting step.

6. Process according to claim 5, further comprising adding magnesium to said copper base alloy prior to said casting

step and said phosphide particle forming step comprising forming at least one of iron phosphide, iron-nickel-phosphide, iron-magnesium-phosphide, nickel-phosphide, and cobalt phosphide particles.

7. Process according to claim 5, further comprising improving mechanical properties of said alloy by adding at least one of aluminum, silver, boron, beryllium, calcium, chromium, indium, lithium, magnesium, manganese, lead, silicon, antimony, titanium, and zirconium in an amount less than 0.1% by weight each prior to said casting step.

8. Process according to claim 1, wherein said copper base alloy contains from about 1.0 to 15% zinc.

9. Process according to claim 1, wherein said copper base alloy contains tin in an amount from about 0.1 to 1.5%.

10. Process according to claim 1, including two homogenization steps, wherein at least one homogenization step is subsequent to a rolling step and wherein the homogenization steps are performed for 2 to 24 hours each.

11. Process according to claim 1, wherein said process anneal is for 1 to 24 hours.

12. Process according to claim 1, wherein said stress relief anneal is for 1 to 20 hours.

13. Process according to claim 1, wherein said casting step forms a strip having a thickness from 0.500 to 0.750

inches and said process further includes milling said strip at least once following said at least one homogenizing step.

14. Process according to claim 1, wherein said cooling step is performed at a cooling rate of 20 to 200° F. per hour until said alloy reaches ambient.

15. A process for making a copper base alloy which comprises the steps of:

casting a copper base alloy containing tin, zinc, iron and phosphorous;

forming phosphide particles uniformly distributed throughout the matrix of said alloy, said particles having a finer component having a particle size in the range of from about 50 to 200 Angstroms and a coarser component having a particle range of from about 0.075 microns to 0.125 microns;

said forming step comprising homogenizing said alloy at least once for at least one hour at a temperature from 1000 to 1450° F., rolling to final gauge including at least one process anneal for at least one hour at 650 to 1200° F. followed by slow cooling, and stress relief annealing at final gauge for at least one hour at 300 to 600° F.

\* \* \* \* \*